

July 5, 1927.

1,634,586

M. KUBO

METHOD OF MANUFACTURING MALLEABLE CAST IRON

Filed June 12, 1922

Fig. 1.



Fig. 3.



Fig. 2.



Fig. 4.



Inventor  
Masakichi Kubo.

B. Singer

Attorney

Patented July 5, 1927.

1,634,586

# UNITED STATES PATENT OFFICE.

MASAKICHI KUBO, OF TOKYO, JAPAN.

## METHOD OF MANUFACTURING MALLEABLE CAST IRON.

Application filed June 12, 1922. Serial No. 567,868.

My invention relates to the process of manufacturing malleable cast iron (including blackheart), and to the provision of a method of producing malleable cast iron with a considerable reduction of cost by decreasing the operating time.

It is well known that malleable cast iron is cast in the form of hard white iron, and given a degree of malleability and toughness by subsequent annealing, during which, either the carbon is partially eliminated, and the remainder left partly as combined carbon, and partly as amorphous or free carbon; or, in the case of blackheart, the amount of the carbon is scarcely altered, but the condition of the bulk of it is changed to amorphous or free carbon and the remainder is left as combined carbon.

In making malleable cast iron, the castings are packed in retorts or annealing pots with oxide of iron (generally hematite ore), put in annealing furnace or oven for heating to a temperature somewhere between 700 degrees C., and the melting point, and kept red hot for several days.

These processes are very expensive, as they need a great deal of fuel, materials, and labor. By means of my invention, I have provided a method of making malleable cast iron from hard white cast iron, without heating the same for a long time as described above.

In carrying out my invention in one form, I have passed an electric current through white cast iron, which is the raw material of malleable cast iron, while buried in oxide of iron, and kept at a temperature of about 900 degrees C., in a gas oven for a short period.

As results I have obtained in a short time a malleable cast iron which has a desirable characteristic malleability and toughness; and unlike the original white cast iron, it can be drilled or bent. According to my experiments with alternating current of 200 amperes per square inch to the section of the material, at a suitable voltage, and a frequency of 50 cycles per second, it was found that almost a complete change in the material may be effected in from one half to one hour, when the thickness of the material is from one quarter to three-eighths of an inch, and the time required was found to decrease as the current density increased.

According to a series of my experiments I declare the facts that the electricity can as-

sist distinctly the elimination or separation of combined carbon in white cast iron if a suitable electric current or voltage be applied while it is kept at a certain high temperature; and an alternating current or voltage is more effective than a direct current or voltage, and also an alternating current of higher frequency is more effective than that of a lower frequency.

In order to explain and to illustrate some of the important applications of my invention, reference will be made to the accompanying drawings, in which:

Fig. 1 is intended to represent diagrammatically an electrical furnace, equipped with the electrodes, for annealing some conical dishes.

Fig. 2 is a gas or oil furnace for treating some white cast iron pieces, with a receptacle for containing hematite.

Fig. 3 is a liquid bath furnace, similar to Fig. 2, for making black-heart castings.

Fig. 4 is a special furnace in which castings are heated electrically.

In Fig. 1, 11 represents walls of the furnace, 13 the hematite ore, 14 the two electrodes, 15 an electric heating unit. As it will be seen the castings 12 are firmly packed in the inner compartment with the hematite

13. In placing the castings an effort should be made to pack them in such a way as to make electrical resistance as uniform throughout as possible. The electrodes 14 are made of iron or other suitable material 90 which can resist chemical action of the hematite 13. Now, the castings 12 and the hematite 13 can be heated by means of the electrical heating unit 15 to a suitable temperature by a proper adjustment of the regulator 16, and a necessary electric current may be passed through the hematite 13 and the castings 12 between electrodes, at a suitable voltage by a proper adjustment of the regulator 17 for a necessary length of time, while the castings 12 are kept at a temperature in the critical range. After this thermal and electrical treatment has been applied, the castings may be taken out at once from the furnace, without keeping them in red hot condition for a long time as usually done.

In Fig. 2, 21 represents the wall and cover of the furnace, built of fire brick, 28 the receptacle made of iron, 23 the hematite ore, 22 the castings, and 25 a gas or oil burner. By means of this arrangement the castings 22 and the hematite 23 may be heated to a

suitable temperature by means of the burner and a necessary electric current may be passed through the castings 22 and the hematite 23 at a suitable voltage for a necessary length of time, which is usually from one half to one hour, by a proper adjustment of the regulator 27. When this malleabilizing process is complete the casting may be removed from the furnace at once.

10 In Fig. 3, 31 represents the wall of the furnace built of fire brick, 38 a crucible, 33 a suitable electrolyte, such as barium chloride, which does not vaporize easily, 34 an electrode, 32 the casting, and 35 the gas or oil burner. By means of the burner the electrolyte 33 and the casting 32 can be heated to a suitable temperature in the critical range, and a necessary electric current may be passed through the electrolyte 33 and the casting 32 at a suitable voltage by a proper adjustment of the regulator 37, to obtain black-heart malleable cast iron castings in a short time.

15 In Fig. 4, 51 represents the wall of a furnace or receptacle made of fire bricks, 53 the hematite ore, 52 the casting of a special form as it will be clear, and 54 the electrodes. As in the present case when a casting has a thick part it happens to be impossible to effect the 20 desirable thermal or electrical treatment by one operation, as in the processes illustrated in Fig. 1, Fig. 2 and Fig. 3, since experiences show that the thicker part of a casting requires, in general, longer time of such a treatment. Therefore, after one operation, as in the process illustrated in Fig. 1, Fig. 2 and Fig. 3, has applied, it is advisable to give the second operation which is intended to be illustrated by the arrangement shown in Fig. 4. Thus, in the second 25 operation, a suitable electric current is sent through the heavier part such as the hub of a wheel, for example, by a proper adjustment of the regulator 57 to heat principally that part of the casting to a temperature in the critical range, in order that that part of the casting may be annealed and electrically treated comparatively in a short time for the purpose of changing the composition of the white cast iron into malleable cast iron which permits drilling or other machining.

30 Thus it is clear that my invention may be conveniently applied for practical purposes, as exemplified above by means of these simple apparatus.

35 The underlying principle involved in this invention seems to be extremely profound and to require a careful study if it is attempted to theorize and to explain the phenomena. In fact it has not been explained or published as far as I know that the separation of carbon from iron carbide compounds, in state of solid at any temperature, can be accelerated by an electric current, although it is a well known fact that the sepa-

ration of carbon from iron carbide compounds in state of fusion, or in state of a chemical solution in a liquid solvent, can be effected or accelerated by an electric current.

40 As stated in the foregoing paragraph, it is extremely difficult to theorize such a delicate intermolecular phenomenon as this. In spite of that, I shall point out and attempt to explain briefly the underlying principle of the fact, as follows:—

45 It is a well known fact that white cast iron is mostly composed of iron and carbide of iron (chemically pure iron and cementite), but when it is heated to a temperature of the critical range, the carbide of iron becomes chemically unstable. Under this condition the molecule seems to be in the state of ionization, having a molecular bipolar condition such that one of the atoms in the molecule has the positive ion and another part has the negative ion, and the amplitudes of both electronic and molecular vibrations within and among the molecules may reach such an extent as to separate carbon atoms from the molecules by molecular vibration and electronic collision, in addition to the action of the separation caused by said bipolar condition. But the rate of the chemical change is exceedingly slow; especially, as it approaches to a point of an equilibrium as a limit, because the effects of the bipolar condition between each molecule manifested by said intramolecular ionization, and of the molecular vibration or electronic collision are feeble when it is treated thermally alone. 50 This seems to be the reason why white cast iron must be heated for a long time, (even several days), at a temperature in the critical range, in order that it may be annealed and made into malleable cast iron.

55 Now, let us imagine that an electromotive force is applied and a natural flow of electric current is effected through the white cast iron for a moment or while thus heated at a temperature in the critical range. Under this condition, the electric current will induce effectively an electromotive force in the molecules, in addition to the thermal action by said electric current, and the free electrons within the molecules will migrate un-

60 der this electromotive force and may speed up to a limit which is a function of the applied electromotive force, and may produce an effective electronic collision, in addition to the molecular vibration, and cause a speedy separation of carbon atoms from the iron carbide molecules and white cast iron may be made into malleable cast iron or blackheart under a suitable condition. And the rate of the chemical change is found to be greater, especially when the applied electromotive force is an alternating one, than when only the electromotive force is applied as described in above, due to the fact that the maximum velocity of the free electrons 65

attained may be much greater, as the crest value of the voltage or current is greater than that of the continuous voltage or current of the same effective value, and electronic movement is then much greater and more effective than otherwise, because the position of the electric potentials change in every half cycle.

In the foregoing an emphasis has been laid on the fact that an alternating electromotive force or electric current is more effective than a continuous electromotive force or electric current. This fact also seems to be, in my opinion, due to the fact that the direction of the applied electromotive force or current changes every half cycle, and when the electric current decreases to zero, the separated carbon which is in the ionic state can change to a neutralized state, and settles to amorphous or free carbon, and when the carbon has settled to the amorphous or free carbon state, it cannot recombine with the iron, because the carbon is changed to graphitic carbon, and the temperature, the current, or voltage, which are used in this process, cannot change the graphitic carbon to the unstable state chemically.

A series of my experimental investigations reveal the facts in addition to the above, that a pulsating voltage or current is more effective than a continuous uniform voltage or current because of the above reasons, and a high frequency alternating voltage or current is more effective than a low frequency alternating voltage or current, because it constitutes the greater number of alternations per second and can give a greater and more effective electronic and magnetic or molecular momentum to accelerate the chemical change within white cast iron.

While I have described the principle of operation of my invention together with apparatus which I now consider to represent the best embodiment thereof, I desire to have it understood that the exact process described and the apparatus shown are merely illustrative and that the invention may be carried out also by other means.

What is claimed is:—

1. The process of converting the combined carbon of white cast iron into uncombined condition without fusion, consisting in en-

veloping the same in a suitable medium, in 55 heating the same to a temperature in the critical range, and passing an electrical current therethrough while thus heated, for the purpose of accelerating the desirable chemical change.

2. The process of manufacturing malleable castings by converting the combined carbon of white cast iron into uncombined condition without fusion, consisting in enveloping the same in a refractory material, 60 in heating the same by fuel or electric heat, to a temperature in the critical range, and passing an electrical current therethrough while thus heated, for the purpose of accelerating the desirable chemical change. 70

3. The process of manufacturing malleable castings by converting the combined carbon of white cast iron into uncombined condition without fusion, consisting in enveloping the same in a suitable medium, such 75 as iron oxide ( $Fe_2O_3$ ) or hematite ore, in heating the same by fuel or electric heat, to a temperature in the critical range, and passing an electric current therethrough, while thus heated, for the purpose of accelerating the desirable chemical change. 80

4. The process of manufacturing malleable castings by converting the combined carbon of white cast iron into uncombined condition without fusion, consisting in enveloping the same in a suitable medium, such as iron oxide ( $Fe_2O_3$ ) or hematite ore, in heating the same with said medium by fuel or electric heat, to a temperature in the critical range, and passing an electrical current therethrough while thus heated, for the purpose of accelerating the desirable chemical change. 90

5. The process of manufacturing malleable castings by converting the combined carbon of white cast iron into uncombined condition without fusion, consisting in enveloping the same in a suitable medium, such as iron oxide ( $Fe_2O_3$ ) or hematite ore in heating the same with said medium, by 95 fuel or electric heat, to a temperature in the critical range, and passing an electrical current through the same and said medium while thus heated, for the purpose of accelerating the desirable chemical change. 100 105

In testimony whereof I affix my signature.

MASAKICHI KUBO.